

March 16, 1926.

1,576,582

V. H. EMERSON

PHONOGRAPH RECORD AND METHOD FOR PRODUCING SAME

Filed Oct. 20, 1920

Fig.1.



Fig.2.



Inventor

V.H. Emerson

By his Attorney

*W.H. Emerson*

Patented Mar. 16, 1926.

1,576,582

# UNITED STATES PATENT OFFICE.

VICTOR H. EMERSON, OF NEW YORK, N. Y.

## PHONOGRAPH RECORD AND METHOD FOR PRODUCING SAME.

Application filed October 20, 1920. Serial No. 418,245.

To all whom it may concern:

Be it known that I, VICTOR H. EMERSON, a citizen of the United States, residing at the city, county, and State of New York, 5 have invented new and useful Improvements in Phonograph Records and Methods for Producing Same, of which the following is a specification.

This invention relates to phonograph records and methods for producing same and has for an object the formation of a composite record, lessening the cost of materials employed, without affecting the record as to its durability or efficiency in sound reproduction.

Considered in its more generic aspect, my improved record and the process for its production relate to the formation of a laminated record having as a body portion a core 20 formed of other than record material, so called, and having the material laid over the top of the record surface of the body portion to the required depth.

For the body portion of my improved record I employ a specifically prepared type of paper composition, and hence broadly considered my invention pertains to two distinct arts, partaking largely of processes employed in the manufacture of papers in the 30 preliminary stages thereof, and also of the art of making phonograph records.

In making paper from wood pulp the first step is to eliminate from the fibrous cellulose foreign materials which comprise the 35 inter-cellular accretions of glutinous, silicious, resinous and other deposits, thus producing the fibre in a relatively pure and strong condition. To this extent my employment of the methods of the paper making art involves nothing novel or materially 40 different from the ordinary processes now in general use. However, having thus produced a fibrous mass of more or less pure cellulose, I re-introduce resin and clay in the required proportions, thoroughly mixing those ingredients with the wood fibre so as to 45 form a homogeneous mass that may be rolled into sheets of the required form and consistency.

In first breaking up the material in order 50 to extract the fibrous portions as free from foreign substances as practicable, and then restoring the resin and clay components which may have been removed in such preliminary processes, a new form of material results which has a uniformly fine texture

that lends itself most effectively to record making, not only as to its strength and toughness, but possessing other properties that enable me to provide a superior record 60 surface.

Having reference to the accompanying drawings, illustrative of a preferred form of my improved record,

Figure 1 is a plan view of a record having 65 a body portion with a superimposed surface of record material, a portion of the top surface having been shown removed; and Fig. 2 is a partial diametral section of the record shown in Fig. 1.

Having reference to the drawings, the numeral 1 represents a preferred form of record produced by my improved process, comprising the body or core portion 2 made of cellulose fibres thoroughly enmeshing the 75 minute particles of clayey materials and resin with which they are combined, as will presently more fully appear.

The body portion 2 of my improved record is first made in sheets from wood pulp having 80 a clay, and preferably silica both, in a finely ground powdered form, and resin soap thoroughly mixed therewith, all of which ingredients are mixed into a uniform homogeneous mass. In obtaining this admixture 85 I employ the cellulose fibre in approximately 70 parts, the resin in 10 parts and the clay and silica in 20 parts, although a slight variation of the portions while affecting the relative properties of the resulting product 90 would produce a phonograph record of varying excellence.

The mass is then rolled into sheets of predetermined thickness in the same manner as paper is ordinarily formed. From the sheets 95 thus prepared the disks may be die-ed out, whereupon the thermoplastic record material is then applied to both sides of the disk 2 when a double faced record is desired, and a sound record groove 4 is impressed in the 100 surface thereof.

Preferably I employ the record material 3 in the convenient form known as record dust, which is spread uniformly to the required depth over the flat surface or surfaces of the disk in the usual manner, and the pressing of the record matrix is likewise performed in the ordinary method now in vogue, in which the required temperature is imparted to the record material in the process of stamping the record. The record material thus by action of the heated matrix 105 110

not only receives the impression of the sound record matrix, but attaches itself to the specially prepared paper disk, forming in the process a most intimate and firm union therewith, owing primarily to the resinous element of the core material.

Heretofore, I am aware, many efforts have been made to obtain laminated records of which a paper base has been employed without attaining to the required degree of efficiency. The paper in the ordinary form of commerce has insufficient hardness or firmness of texture to stand up under the impression pressure, but reacts after the stress of stamping is removed and an imperfect record results.

To overcome this specific difficulty various schemes have been employed to render more rigid and less compressible the paper material thus employed, especially porous types of paper having been employed in certain instances, the manufactured paper body being taken in substantially its finished form for the initial step of all such processes.

However, by my improved process I take the unformed cellulose fibres obtained in the same manner as in making paper and, as already pointed out, thereto add the stiffening and sizing elements as above in a form that renders them peculiarly adaptable to a perfect union with the fibrous cellulose. That is to say, I employ the resin in the proportion mentioned first dissolved preferably in an alkali solution. Then the powdered clay in suitable proportions is incorporated therewith, the two in turn being thoroughly mixed with the cellulose pulp until the clayey and silica components are thoroughly bound to the fibres of the cellulose ingredient. When the combining process has been carried on to the required extent a uniform homogeneous fibrous material results, modifying the natural pliability of the cellulose fibre by means of the added qualities of the rigidity and stiffness of the clay and silica components having been introduced in the proper proportions to produce the required stiffness.

The resulting product is then rolled into sheets of the desired thickness in the usual manner, then cut into disks of the required diameter, preferably by dieing, the central orifice being usually inserted by the dieing out process. The disk thus prepared receives upon its flat surface a thin layer of thermoplastic record material, dusted on in the ordinary way, in which the record material in that form is applied, and with the record material thus adhering to the surfaces of the paper disk, the article is inserted in the usual stamping press wherein the matrix is brought to the required temperature to cause the thermoplastic record material to flow, in which condition it

makes a permanent, lasting cleavage with the paper impregnated with the resin binder which as has been described serves also to unite the clayey and other particles with the cellulose fibres. At the same time the presence of the clayey particles furnishes sufficient rigidity to the body member 2 so that the full impression of all the irregularities produced in the recording of the sound are fully and minutely imprinted and recorded in the groove thus formed in the record material. Furthermore, the presence of the silica particles is so completely and uniformly distributed throughout the entire body portion of the paper core as to prevent the paper from yielding under the pressure of the stamping process, thereby becoming distorted, later to re-form and otherwise affect disastrously the sound record impressed in the record material thereon.

I am aware that various efforts have been made thus to impregnate the texture of the ordinary paper, to this end some of the more porous types of blotting paper having been employed. But in all known processes by which this object was sought to be attained, it has been found upon investigation that portions of the paper had received the ingredients in excess proportions, while other parts received an insufficient portion of the sizing material, the paper body or core remaining comparatively soft and spongy. Therefore it is an important feature of my present invention that I am able at the outset to produce a perfectly uniform homogeneous core member to which the record layer will make a permanent union and will receive a perfect record, even to the minutest undulatory detail thereof.

Having described my invention, what I claim is:

1. A tablet having a body member of nonrecord material, containing in uniform arrangement throughout its body in predetermined proportions silica clay and resin, having upon the surface a layer of thermoplastic record material with a sound record therein.

2. A tablet having a body portion of specially prepared paper board containing in predetermined proportions silica clayey material and resin and a thermoplastic record layer thereon having a sound record recorded therein.

3. A method of making phonograph records by my improved process which consists in first preparing a cellulose pulp substantially free from other materials, adding thereto a resin solution containing silica in substantially the proportions of ten parts of resin, twenty parts silica, seventy parts of cellulose pulp, thoroughly mixing the same to form a homogeneous material, then rolling into sheets of predetermined thick-

ness, drying and stamping therefrom disks of suitable size and lastly impressing thereon by means of heated matrices a layer of thermoplastic material having a sound record groove therein.

4. A process for making tablets for sound records which consists in first providing a pulp of cellulose fibre, removing therefrom all resinous and other foreign sub-

stances, adding in predetermined portions 10 resin in solution, having clayey material also in solution, forming the pulp thus prepared in sheets of suitable thickness, and stamping therefrom disks of the required diameter for records to be made thereupon. 15

In testimony whereof I have hereunto set my hand.

VICTOR H. EMERSON.